

## UNITED STATES PATENT OFFICE

2,661,296

## RUST INHIBITING COMPOSITION

Knapel F. Schiermeier and Herbert A. Poitz,  
Alton, Ill., assignors to Shell Development Company, San Francisco, Calif., a corporation of Delaware

No Drawing. Application April 26, 1948,  
Serial No. 23,398

5 Claims. (Cl. 106—14)

1

This invention relates to an all purpose corrosion inhibiting composition. More particularly, this invention pertains to corrosion inhibiting compositions having the ability of displacing moisture, corrosive materials and the like from metal surfaces and forming thereon a tenacious protective film, which is impervious to moisture and other contaminants.

It is well known that moisture, corrosive fluids and gases, e. g. H<sub>2</sub>S, SO<sub>2</sub>, etc. readily attack not only metallic surfaces but non-metallic surfaces and cause corrosion, rusting, pitting and other damages to such surfaces. Also aqueous solutions when in contact with a metallic surface readily attack it and cause corrosion and rusting. Under certain conditions the problem of corrosion becomes exceedingly serious because once started it becomes progressively accelerated. Thus, oils containing small amounts of water, become very corrosive to contacting metals. This is due to the fact that oils and particularly liquid petroleum hydrocarbons are relatively good solubilizers of oxygen and any moisture present therein becomes surrounded by an almost inexhaustible store of oxygen. Moisture under such conditions is inhibited from evaporating and since the rate of transfer of oxygen from hydrocarbons, such as mineral oil or gasoline, to water is limited, ideal conditions for rusting and corrosion are set up. The presence of electrolytes and formation of corrosive decomposition products in oils and the like also greatly increase the rate of corrosivity.

Under conditions where, in addition to those enumerated, elevated temperature is encountered, corrosion activity is greatly accelerated. Thus, moisture, salt sprays and other contaminants or acidic composition products and corrosive gases formed during operation of engines, such as internal combustion engines, diesel engines, aircraft engines, turbines and various other machinery and industrial equipment, readily attack and rust or corrode contacting metal surfaces. The damage thus caused is not to the metal surface alone for rust particles frequently break off and enter the circulating system of engines and cause plugging, clogging, and fouling of conduit lines, columns, plates, and the lines of cracking equipment, tubes, evaporators, etc.

Corrosion of alloyed bearings and other alloyed surfaces due to contact with water can attain such an aggravated stage as to cause great fatigue stresses to be set up, which ultimately results in cracking of the metal.

The problem is equally serious when combating rusting and corrosion of steel drums, stor-

2

age tanks used to store gasoline, hydrocarbon oils and the like. Moisture adhering to pickled steel, quenched steel, equipment such as instruments, engine starters and generators on landing crafts, hydraulic systems, machinery for metal processing and the like are also extremely susceptible to corrosion and must be protected. The problem is particularly serious when metallic parts, machines, e. g. aircrafts and the like are transported over bodies of salt water over long periods of time under humid and high temperature conditions. Unless the metal surfaces are protected with a coating composition which is impervious to active corrosion producing agents, serious and damaging corrosion sets in.

Such contaminants also have a detrimental effect upon the medium in which they are dispersed. In lubricating and liquid fuel mediums they cause oxidation, interfere with the functioning of additives or decrease their efficiency, form emulsions and thickening of the fluid and generally cause gumming and sticking of movable parts.

Countless materials and compositions have been tried for protecting surfaces by forming on said surface a non-reactive corrosion protective film having lubricating properties. Metal surfaces have been coated or treated with greases, fatty compositions, waxes, organic compounds, e. g. organic acids, amines; inorganic compounds and the like in order to protect them against corrosion. In almost all cases where no chemical reaction occurred between the surface treated and the corrosion or rust inhibitor very little benefit was derived. This is due to the fact that non-chemical reactive inhibitors are incapable of penetrating the surface being protected and are incapable of displacing the contaminant therefrom. In cases where such inhibitors are able to form protective coatings on surfaces they are easily displaced by moisture or rupture readily. They are relatively ineffective against corrosive acidic materials and no gases such as are formed during operation of combustion and turbine engines and are easily destroyed when applied to surfaces which are subjected to high temperatures.

It has now been discovered that various metallic surfaces can be protected against corrosion by coating said surfaces with a composition comprising a major amount of a liquid base such as an aromatic solvent or a blend of an aromatic solvent and a light liquid hydrocarbon having a boiling point not exceeding around about 650° F. 55 said liquid base containing a substantial amount

of a waxy hydrocarbon and a minor amount of a heavy metal salt of an organic cyclic acid.

The aromatic solvents may be obtained by any suitable means such as the treatment of petroleum products with various selective solvents or mixtures of solvents which are adapted to segregate the relatively more aromatic constituents from the non-aromatic constituents. Suitable solvents may be represented by sulfur dioxide, phenol, furfural, nitro-benzene, cresol, aniline, beta, beta dichloro-diethyl ether and the like. Hydrocarbons which are particularly suitable for treatment with above type of solvents are petroleum hydrocarbons having a boiling range of from about 300° F. to about 600° F. and may be specifically represented by kerosene, gas oil, light hydrocarbon oil fractions and the like. Particularly preferred are aromatic solvents obtained by the sulfur dioxide treatment of a 300° F. to 370° F. petroleum hydrocarbon cut according to the well known Edeleanu process. Characteristics of aromatic solvents obtained by subjecting kerosene to the Edeleanu process are given below.

|                                         |               |
|-----------------------------------------|---------------|
| Gravity, °API, at 60° F-----            | 35.3-35.2     |
| Spec. gravity, 60/60° F-----            | 0.8438-0.8483 |
| Flash Tag, cc., °F-----                 | 119-112       |
| Aniline pt., °F. ASTM-----              | 9.0-31        |
| Aromatics, ASTM, percent weight-----    | 58-58         |
| Alkyl phenols (SMS .246)-----           | 11-15         |
| Aromatic free residue, tool-----        | 32-42         |
| Naphthenes, mol percent, Maltiello----- | 61-63         |
| Paraffins-----                          | 37-39         |

Aromatic solvents suitable for use as a component of compositions of this invention may be obtained by other means than solvent extraction of petroleum distillates. Thus aromatic solvents may be obtained from catalytic conversion of petroleum hydrocarbons such as obtained from recycle stocks from catalytic cracking. Also aromatics such as naphthalene, fluorene, phenanthrene anthracene, coal tar residues and the like, may be admixed in small amounts with aromatic solvents of the type described above.

The aromatic solvents should comprise at least about 45% of the composition. If desired part of the aromatic solvent may be replaced with a light liquid hydrocarbon fraction and/or fractions providing the aromatic solvent constitutes a major proportion of the blend and the light liquid hydrocarbon constitutes a minor proportion of the blend. Generally the aromatic solvent comprises at least two-thirds of the mixture when blended with a light hydrocarbon. Preferably the aromatic solvent is used as the sole carrier, or diluent for additives of this invention.

The light liquid hydrocarbon fractions which may be blended with aromatic solvents may be obtained from any type of petroleum base such as paraffinic, naphthenic, asphaltic and/or their fractions. The fractions desired are those normally liquid fractions which have a boiling point range below that of lubricating oil. Specific liquid hydrocarbons which may be obtained from petroleum distillate by any suitable means include, kerosene, mineral seal oil, mineral spirits, light spindle oil, light spray oils, petroleum solvent naphtha as well as various other petroleum naphtha cuts, petroleum ethers, octane, isooctane, dodecane, cycloparaffins, e. g. cyclohexane, methylcyclohexane, etc.

To an aromatic solvent or to a blend of an aromatic solvent and a hydrocarbon as described above which generally comprises at least 50%

of the composition of this invention is added between about 15% to 30% and preferably between about 20 to 30% of a waxy hydrocarbon such as paraffin wax, petrolatum and the like.

The waxy hydrocarbon should be substantially non-aromatic and may be derived from petroleum fractions such as petroleum distillates or residues, or the waxy hydrocarbons may be produced synthetically by polymerization of olefinic materials such as by the Fischer-Tropsch process or by dehydration of long chain aliphatic alcohols.

Waxy hydrocarbons may be recovered from suitable petroleum fractions such as Pennsylvania crudes, East Texas crudes, Mid-Continent crudes and the like by de-asphaltizing the hydrocarbon and thereafter removing the wax from the asphalt free hydrocarbon fraction by any known suitable means.

In the solvent process a solvent is selected in which the oil is relatively soluble but in which the asphaltic materials are relatively insoluble. Among such solvents are the light liquid hydrocarbons such as ethane, propane, butane, as well as naphtha and gasoline. The wax-oil mixture may be removed from the asphalt-free solution by chilling the solution, and then separating the precipitated wax by settling, filtering, or centrifuging. Waxy materials thus produced are known in the art as slop waxes, petrolatum stock, slack waxes, scale waxes, paraffin waxes, plate malocrystalline and needle waxes, micro-crystalline waxes and the like. The waxes are differentiated from each other by the degree of deoiling to which they are subjected and all of them may be used provided they are substantially free from aromatics.

De-waxing or separation of the above waxy constituents from the oil may be accomplished by selective solvent treatment using as the diluents liquified normally gaseous hydrocarbons such as propane, butane and other corresponding olefins and/or their mixtures as well as oxygen-containing liquid organic substances such as alcohols, ethers, esters, ketones, aldehydes, acids and/or their mixtures. These may include methyl, ethyl, propyl, butyl, amyl alcohols, methyl or methylethyl ether; acetone, diethyl, dimethyl, methylethyl, methylisobutyl ketones and the like. Chlorinated hydrocarbons such as carbon tetrachloride or trichloroethylene and mixtures of chlorinated and non-chlorinated hydrocarbons as mentioned above also may be used.

The first step in obtaining waxy constituents from petroleum crudes for example such as Mid-Continent crude is to treat said crude with about six volumes of liquid propane so as to remove the asphalt. The propane from the propane-oil solution is vaporized so that the ratio of propane to oil is reduced approximately 2 to 1. The solution is then chilled to about -40° F. and lower causing separation of the wax from the oil. The wax can be removed by filtration and the propane separated from the de-asphalted and dewaxed oil and waxy material by distillation.

Waxy materials can also be recovered from distillate or residuum lube oil fractions and these wax fractions can be split still further into special wax cuts having desired characteristics by use of selective solvents. This is based on a difference in solubility of different waxy fractions in a given solvent. Thus, when using a methylethyl ketone type solvent the aromatic

constituents can be removed by successively cooling the mixture down to between about -40° F. and -70° F. so as to remove the aromatics which become substantially soluble in the solvent as the temperature is lowered while the straight chain waxes and isoparaffins become substantially insoluble in the solvent. The straight chain waxes can be separated from the isoparaffins by extraction and fractional crystallization. Depending upon the distillate cut used waxes of from 12 to above 36 carbon atoms and higher can be obtained.

Instead of obtaining natural waxy materials from petroleum fractions, straight chain waxes can be produced synthetically by polymerization of olefins under pressure of dehydrating long chain fatty alcohols such as octadecyl alcohol and the like. Mixtures of the above-mentioned waxes may be used in compositions of this invention. If desired, the waxy hydrocarbon may be oxidized by any suitable means.

The final essential ingredient which comprises a component part of compositions of this invention is a lead salt of an organic cyclic acid said salt, e. g., lead naphthenate being present in an amount of between about 10 to 25% and preferably between about 18 to 22% by weight.

Cyclic acids which may be used to form the heavy metal salts may be represented by the formula  $R(Y)_a(Z)_b(CXXH)_c$ , wherein R is a cyclic radical; the X's may be O, S, Se and/or Te; the acid radical (CXXH) being linked directly or indirectly to R; Y is a polar group; Z is an organic radical from the groups consisting of alkyl, alkylene, alkylaryl, aryl alkyl, alkoxy, aroxyl, aryl radical and the like; a and b may be zero or an integer of 1 or 2, and c is an integer of 1 or 2. The substituent group represented by Y in the formula may be hydroxy, amine, nitro, nitroso, halogen, sulfo, mercapto, and the like. The polar group or groups may be attached directly or indirectly to the R radical.

Specifically cyclic acids may include: naphthenic acid (derived from petroleum hydrocarbons), phenyl naphthenic acids, hydroxy-phenyl naphthenic acids, benzyl naphthenic acids, benzoyl naphthenic acids; naphthyl naphthenic acids, xenyl naphthenic acids, phenyl vinaconic acid, phenyl caronic acid, truxillic acids, phenyl morphinic acid, phenyl-pinic acid, phenyl camphoric acid, phenyl camphenic acid, phenyl 2,3,4-trimethyl cyclopentane-3-carboxylic acid, phenyl hexahydrobenzoic acids, hydrophenyl hexahydrobenzoic acids, benzoyl hexahydrobenzoic acids, naphthyl hexahydrobenzoic acids, phenyl hexahydrophthalic acids, phenyl quinic acid, hexahydrobenzoic acid, tetrahydrophthalic acid, hexahydrophthalic acid, tetrahydrotoluic acid, alkyl hexahydrophthalic acid, alkylene cyclohexadiene carboxylic acid, cyclohexane carboxylic acid, cyclohexylacetic acid, cyclohexylbutyric acid, cyclohexyl caproic acid, cyclohexylpropionic acid, cyclohexylvaleric acid, fencholic acid, cholic acid, abietic acid, etc.

The salts of this invention may be obtained by reacting an organic cyclic acid or mixtures of said acids with an oxide, carbonate, sulfide and the like of lead.

Some specific salts of organic cyclic acids are listed below in which the lead cation part may be combined with any of the anion parts listed to form organic salts of this invention

#### Anion part

Petroleum naphthenic acid

- Phenyl naphthenic acid
- Hydroxyphenyl naphthenic acid
- Naphthyl naphthenic acid
- Phenyl vinaconic acid
- Phenyl binic acid
- Phenyl hexahydrobenzoic acid
- Phenyl hexahydrophthalic acid
- Tetrahydrotoluic acid
- Cyclohexadiene carboxylic acid
- Cyclohexyl caproic acid
- Abietic acid

If desired, various additives may be added to compositions of this invention to improve its properties. Among such additives may be included organic amines and amine salts e. g. aliphatic cycloaliphatic, alkyl amines such as octadecylamine, cyclohexylamine, dicyclohexylamine, methyl cyclohexylamine, triethanolamine; paraffine oleate, dicyclohexylamine oleate; salts of inorganic acids, e. g. metal phosphates, methyl oleyl aluminum phosphates; organic esters, e. g. dilorol phosphate, dilauryl phosphate, polycarboxylic acids, e. g. alkyl succinic acid; inorganic compounds, e. g. sodium nitrite, lithium nitrile, sodium chromate, etc. The amount of these additives is generally added in an amount not exceeding 5% and preferably 1 to 3% is usual.

A general formula of a composition of this invention may consist of the following components by weight.

|                                                                                    | Broad Range | Limited Range |
|------------------------------------------------------------------------------------|-------------|---------------|
| 35 Waxy hydrocarbon                                                                | 20-35%      | 25-30%        |
| Lead salt of an organic cyclic acid                                                | 10-25%      | 18-22%        |
| Optional additive, e. g. amines, petroleum sulfonate                               | 0-5%        | 1-3%          |
| Aromatic solvent and/or mixture of aromatic solvent and a light liquid hydrocarbon | balance     | balance       |

Specific examples of a preferred composition (henceforth designated as composition A, B, C, D), of this invention comprises:

| Composition A            |         |
|--------------------------|---------|
| Lead naphthenate         | 18-22   |
| Short residue petrolatum | 25-30   |
| Aromatic solvent         | balance |

| Composition B            |         |
|--------------------------|---------|
| Lead naphthenate         | 10-20   |
| Short residue petrolatum | 20-30   |
| Cyclohexylamine          | 1-5     |
| Aromatic solvent         | balance |

| Composition C                     |         |
|-----------------------------------|---------|
| Lead naphthenate                  | 10-15   |
| Oxidized short residue petrolatum | 20-25   |
| Cyclohexylamine                   | 1-5     |
| Calcium petroleum sulfonate       | 1-5     |
| Aromatic solvent                  | balance |

| Composition D                     |         |
|-----------------------------------|---------|
| Lead naphthenate                  | 10-20   |
| Oxidized short residue petrolatum | 20-30   |
| Calcium petroleum sulfonate       | 1-5     |
| Aromatic solvent                  | balance |

Compositions of this invention may be prepared by adding at about 180° F. waxy hydrocarbon such as petrolatum to a lead base or the like and mixing the two at this temperature for about 15 minutes. The mixture is then slowly cooled under agitation to around about 135° F. at which point

the aromatic solvent is slowly added. The mixture is then reheated to about 120° F. until a homogeneous composition is obtained and cooled to room temperature with continuous agitation.

In order to determine the protective properties compositions of this invention possess, various metals were coated with compositions of this invention and subjected to the following tests.

#### *Humidity cabinet test*

In this test sandblasted or polished steel panels which have been coated with a product of this invention were exposed continuously in an atmosphere of 100% relative humidity at a constant temperature (100° or 120° F.). A slow flow of saturated air through the cabinet is maintained and moisture condenses on the panels. The average time of exposure until rusting occurs on the faces of the panels is taken as the life of the coating.

#### *Salt spray test*

In this test polished steel panels which have been coated with a desired product to be evaluated are exposed continuously at a constant temperature (95° or 100° F.) to a salt mist or fog which is produced by the atomization of a 20% sodium chloride solution. The average time until rusting occurs on the faces of the panels is taken as the life of the coating.

#### *Ultraviolet weathering unit test*

In this test polished or sandblasted steel panels which have been coated with a desired product to be evaluated are continuously exposed to intense light from a carbon arc and are intermittently wetted by a fine water spray. The average time until rusting occurs on the faces of the panels is taken as the life of the coating.

#### *Unsheltered, sheltered, outdoor and indoor exposure test*

In the unsheltered outdoor exposure test, polished or sandblasted steel panels which have been coated with a desired product to be evaluated are fastened on uncovered racks facing south at an angle of 45 degrees from the vertical and are exposed continuously until rusting occurs. The average exposure time of tests conducted during different seasons of the year indicates the actual life of the coating. For sheltered outdoor exposure panels are suspended in a cabinet which is open to the atmosphere from the sides or bottom, but the panels are completely protected from rain, snow, etc. Indoor exposure test is designed to determine the protective properties products possess in resisting fluctuation in temperature and relative humidity.

Composition A as noted in column 6 of this invention having the following properties was subjected to the above tests and the results are as tabulated below:

#### *Properties of Composition A*

|                                        |      |
|----------------------------------------|------|
| Gravity at 60° F. API                  | 26.1 |
| Flash, °F. (COC)                       | 134  |
| Viscosity at 100° F. Saybolt Universal | 59   |
| Pour point, °F.                        | 40   |

#### *Test results*

|                                     |            |
|-------------------------------------|------------|
| Humidity cabinet, hrs.              | Over 1000  |
| Salt spray, 20%, hrs.               | 280        |
| U-V weathering unit, hrs.           | Over 300   |
| Unsheltered outdoor exposure, days. | Passed 120 |
| Sheltered outdoor exposure, mos.    | 12-24      |
| Indoor exposure, mos.               | Over 24    |

The above Composition A was far superior to the best known commercial product (X) which when subjected to some of the above desired tests gave the following results:

|   |                                     |           |
|---|-------------------------------------|-----------|
| 5 | Salt spray, 20% hrs.                | 160       |
|   | Weathering unit, hrs.               | 90        |
|   | Unsheltered outdoor exposure, days. | Failed 14 |

10 Compositions of this invention may if desired, be very easily removed by flushing, wiping or any other suitable means. Compositions of this invention may also be applied to non-metallic surfaces which require protection against corrosion, moisture, the elements and the like.

15 Many modifications and variations of this invention as hereinbefore set forth may be made without departing from the spirit and scope thereof and therefore only such limitation should be imposed as indicated in the appended claims.

20 We claim as our invention:

1. A rust inhibiting composition of matter consisting essentially of the following constituents in the following proportions:

|                          | Per cent by weight |
|--------------------------|--------------------|
| Lead naphthenate         | 15-25              |
| Short residue petrolatum | 25-30              |
| Aromatic solvent         | Balance            |

30 2. A rust inhibiting composition of matter consisting essentially of the following constituents in the following proportions:

|                          | Per cent by weight |
|--------------------------|--------------------|
| Lead naphthenate         | 15-25              |
| Short residue petrolatum | 20-30              |
| Cyclohexylamine          | 1-5                |
| Aromatic solvent         | Balance            |

40 3. A rust inhibiting composition of matter consisting essentially of from about 15 to 35% of a petroleum wax, from about 10 to 25% of lead salt of naphthenic acid and the balance being an aromatic solvent.

45 4. A rust inhibiting composition of matter consisting essentially of a major proportion of an aromatic solvent, a minor amount of about 30% of a petroleum wax, and about 20% of lead salt of naphthenic acid.

50 5. A rust-inhibiting composition of matter consisting essentially of the following constituents in the following proportions:

|                          | Per cent by weight |
|--------------------------|--------------------|
| Lead naphthenate         | 18-22              |
| Short residue petrolatum | 25-30              |
| Aromatic solvent         | Balance            |

KNAPEL F. SCHIERMEIER.  
HERBERT A. POITZ.

#### *References Cited in the file of this patent*

#### *UNITED STATES PATENTS*

| Number    | Name            | Date          |
|-----------|-----------------|---------------|
| 2,060,138 | Taylor          | Nov. 10, 1936 |
| 2,124,446 | Detwiler        | July 19, 1938 |
| 2,182,992 | Lebo            | Dec. 12, 1939 |
| 2,184,952 | Zimmer et al.   | Dec. 26, 1939 |
| 2,334,071 | Cook et al.     | Nov. 9, 1943  |
| 2,348,715 | Adams et al.    | May 16, 1944  |
| 2,359,946 | Sudholz et al.  | Oct. 10, 1944 |
| 2,415,353 | Johnston et al. | Feb. 4, 1947  |